

## UNITED STATES PATENT OFFICE

2,356,647

## SAFETY FUEL

Cecil L. Brown, Baton Rouge, La., assignor to  
Standard Oil Development Company, a corpora-  
tion of Delaware

No Drawing. Original application December 7,  
1938, Serial No. 244,357, now Patent No.  
2,321,280, dated June 8, 1943. Divided and this  
application July 22, 1942, Serial No. 451,947

9 Claims. (Cl. 44—80)

This application is a division of copending ap-  
plication Serial No. 244,357, filed December 7,  
1938, now Patent No. 2,321,280, dated June 8,  
1943.

The present invention is directed to fuels for  
air craft, known as safety fuels.

Safety fuels are characterized by a high flash  
point, a high octane number, good volatility and  
gum stability. For example, a good safety fuel  
should have a Tag closed cup flash point of 100°  
F. or more, an octane number of about 100, and a  
boiling range of about 300—400° F. It should  
have also the other characteristics of good avia-  
tion gasoline, such as a good gum stability and  
a good break down test.

The desirability of using a safety fuel has long  
been apparent in the aviation industry. Thus  
far, however, the industry has not universally  
adopted any standard safety fuel, primarily be-  
cause there has been no available source of sup-  
ply of such fuels at a suitable price.

It has hitherto been proposed to produce safety  
fuels by several methods such as the destructive  
hydrogenation of selected distillates or crudes,  
the extraction with sulfur dioxide of certain dis-  
tillates or crudes, and the catalytic cracking un-  
der selected conditions of such extracts. The  
fuels produced by the first method are rather  
high priced due to the limited quantity of suit-  
able raw materials. The fuels produced by the  
latter two methods have so low an initial octane  
number and so low a lead susceptibility that the  
amount of lead required to convert them into 100  
octane fuels makes their cost well-nigh prohib-  
itive.

I have now found that fuels having satisfactory  
characteristics for safety fuels such as high ini-  
tial octane number, high lead susceptibility and  
suitable boiling range can be produced from C<sub>4</sub>  
iso-hydrocarbons. For example, the copolymer-  
ization of normal and isobutylene yields a heavy  
hydrocarbon fraction which, when hydrogenated,  
boils between about 300 and 385° F., has a  
high flash point and a high octane number.

I have found that by cutting the mixture of  
hydrocarbons produced by the reaction between  
an isoparaffin and an olefin, such as isobutane  
and normal or isobutylene, at about 300° F., it is  
possible to produce a heavy fraction having a  
boiling range of from about 300 to 400° F. which  
has a Tag closed cup flash in excess of 100° F.,  
a high initial octane number, and a high lead  
susceptibility. A particularly desirable safety  
fuel, according to the present invention, is a  
blend of the last mentioned heavy fraction of

alkylation product with hydrogenated tri-isobu-  
tylenes boiling between about 330 and 380° F., with  
the latter constituting from 10 to 50% of the  
blend.

The basic materials for the safety fuels of the  
present invention are available in large quanti-  
ties and the methods by which they are converted  
into the desired safety fuels are not costly. For  
example, practically all refinery gases resulting  
from cracking processes of various types con-  
tain substantial percentages of isobutylene and  
normal butylene which can be caused to copoly-  
merize by being contacted with sulfuric acid of  
a strength ranging from 60 to 75% at a temper-  
ature between about 175 and 250° F. This  
process is usually conducted with a view of pro-  
ducing dimer, and to this end it may be desir-  
able to recycle trimer to the reaction chamber.  
As the result of the present invention, this proc-  
ess can be carried out with a view of producing  
the highest yield per pass of high boiling hydro-  
carbons, whereby the efficiency of the method is  
increased.

There are large reservoirs of isobutane which  
can be utilized as sources of raw material for  
the second embodiment of the present invention.  
The reaction between isobutane and the  
olefins of refinery gases proceeds with ease at  
normal room temperatures in the presence of  
concentrated sulfuric acid. This reaction, which  
yields a product containing C<sub>5+</sub> hydrocarbons,  
can be made to yield substantial amounts of a  
product boiling within the safety fuel range by  
recycling C<sub>5</sub>-C<sub>8</sub> hydrocarbons to the reaction  
zone.

The fuels of the present invention do not per-  
se have an octane number of 100. The co-poly-  
mer of isobutylene and normal butylenes, when  
hydrogenated, has an octane number of about  
90 which can be brought to 99.5 with 3 cc. of tet-  
raethyl lead per gallon. Likewise, the high boil-  
ing alkylation fraction, especially when blended  
with about 40% of hydrogenated triisobutylene,  
has a clear octane number of about 90 which  
can be raised to 100 with 3 cc. of tetraethyl lead  
per gallon.

The safety fuel of the present invention is pref-  
erably composed entirely of the reaction product  
of an iso-C<sub>4</sub> hydrocarbon with a different C<sub>4</sub> hy-  
drocarbon. It may be mentioned, however, that,  
when the fuel is an alkylation product, it may be  
produced from isopentane or isohexane as well  
as from isobutane. Likewise, olefins other than  
the butylenes may be employed. In any case, the  
fuel, as previously mentioned, may contain sub-

stantial quantities of hydrogenated triisobutylene. Other suitable blending agents are alkylated aromatics boiling between 300 and 400° F. Typical examples of such alkylated aromatics are ethyl benzene, propyl benzene, isopropyl benzene, methyl benzene, *o*, *m*, *p*, trimethyl benzene, 1, 2, 3, trimethyl benzene 1, 2, 4, trimethyl benzene, 1, 3, 5, secondary butyl benzene, isobutyl benzene, tertiary butyl benzene, and methyl isopropyl benzene, *p*.

Alternatively, a fraction boiling between 300 and 400° F. of the product resulting from the alkylation of aromatics with olefins may be employed.

The characteristics of typical examples of aviation safety fuel according to the present invention are given in the following table. Fuel A of this table was prepared by reacting isobutylene and normal butylene in the presence of sulfuric acid of a strength of about 70% at a temperature of 170° F., recovering from the product a fraction boiling above 300° F. and hydrogenating this fraction by contacting it with a catalyst composed of  $\text{MoO}_3$ ,  $\text{ZnO}$  and  $\text{MgO}$  at a temperature of 500–600° F. and under a pressure of 3000 pounds per square inch in the presence of a large excess of hydrogen.

Fuel B was prepared by reacting isobutane and the iso- and normal butylene in C<sub>4</sub> refinery cut in the presence of sulfuric acid having a strength of 98% at a temperature of 70° F. and under a pressure sufficient to maintain the reactants in the liquid state and recovering from the product a fraction having the boiling range shown in the table.

Fuel C was prepared by blending with fuel B hydrogenated triisobutylene boiling between 330 and 358° F., the latter constituting 40% of the blend.

|                             | Fuel A  | Fuel B   | Fuel C   |
|-----------------------------|---------|----------|----------|
| A. P. I. gravity            | 52.7    | 55.8     | 55.8     |
| Color Saybolt               | +19     | +26      | +27      |
| Aniline point               | °F      | 182      | 189      |
| Sulfur                      | percent | 0.01     | 0.008    |
| Doctor                      |         | Passes   | Passes   |
| Corrosion, cu. dish         |         | Passes   | Passes   |
| Gum, cu. dish               | mgs     | 3.6      | 3.8      |
| Acid heat                   | °F      | 2        | 1        |
| Bromine No.                 |         | 3        | 1        |
| Flash, Tag closed cup       |         | 112      | 103      |
| Reid vapor pressure         |         | Below 1# | Below 1# |
| Army octane number          |         | 89.4     | 77.0     |
| Army octane number +3.0 co. |         | 99.5     | 96.4     |
| TEL                         |         |          |          |
| Initial                     | °F      | 304      | 323      |
| 6%                          |         | 319      | 336      |
| 10%                         |         | 324      | 341      |
| 30%                         |         | 336      | 351      |
| 50%                         |         | 345      | 357      |
| 70%                         |         | 352      | 363      |
| 90%                         |         | 362      | 373      |
| Final                       | °F      | 384      | 393      |
| Recovery                    | percent | 98.0     | 98.0     |
| Residue                     | do      | 1.0      | 1.0      |

The nature and objects of the present invention having thus been described, what is claimed as new and useful and is desired to be secured by Letters Patent is:

1. A safety fuel boiling substantially completely between about 300° F. and about 400° F., having a flash point of at least 100° F. by the closed cup method, composed predominantly of a mixture of paraffinic reaction products of an isoparaffin and an olefin and also containing compounds formed by hydrogenating the normally liquid condensation product of C<sub>4</sub> olefins said product boiling within the above-stated range,

said mixture containing also sufficient anti-knock agent to raise its octane number to 100.

2. A safety fuel boiling substantially completely between about 300° F. and 400° F., having a flash point of at least 100° F. by the closed cup method, composed predominantly of a mixture of paraffinic reaction products of an isoparaffin and an olefin and compounds formed by hydrogenating the condensation product of normal and isobutylenes said product boiling within the above-stated range and said mixture containing sufficient anti-knock agent to raise its octane number to about 100.

3. A safety fuel boiling substantially completely between about 300° F. and 400° F., having a flash point of at least 100° F. by the closed cup method, composed of a mixture of hydrogenated tri-butylene said product boiling within the above-stated range and paraffinic reaction products of an isoparaffin and an olefin, and containing sufficient anti-knock agent to bring its octane number to about 100.

4. A safety fuel according to claim 3 in which hydrogenated tri-isobutylenes boiling between about 330° F. and about 380° F. constitute from about 10 to about 50% of the mixture.

5. A safety fuel boiling substantially completely between about 300° F. and about 400° F., having a flash point of at least 100° F. by the closed cup method, composed predominantly of a mixture of paraffinic reaction products of isopentane and an olefin and compounds formed by hydrogenating the normally liquid condensation products of C<sub>4</sub> olefins said products boiling within the above-stated range, said mixture containing sufficient anti-knock agent to raise its octane number to about 100.

6. A safety fuel boiling substantially completely between about 300° F. and about 400° F., having a flash point of at least 100° F. by the closed cup method, composed predominantly of a mixture of paraffinic reaction products of isopentane and an olefin and compounds formed by hydrogenating the normally liquid condensation products of isobutylene said products boiling within the above-stated range, said mixture containing sufficient anti-knock agent to raise its octane number to about 100.

7. A safety fuel boiling substantially completely between about 300° F. and about 400° F., having a flash point of at least 100° F. by the closed cup method, composed predominantly of a mixture of paraffinic reaction products of isopentane and an olefin and compounds formed by hydrogenating triisobutylene, said mixture containing sufficient anti-knock agent to raise its octane number to about 100.

8. A safety fuel boiling substantially completely between about 300 and 400° F., having a flash point of at least 100° F. by the closed cup method, composed of hydrogenated triisobutylene and the paraffinic compounds formed by the reaction between isobutane and a C<sub>4</sub> olefin, and containing sufficient anti-knock agent to bring its octane number to about 100.

9. A safety fuel boiling substantially completely between about 300° and 400° F., having a flash point of at least 100° F. by the closed cup method, composed of hydrogenated triisobutylene and paraffinic compounds formed by the reaction between isobutane and isobutylene, and containing sufficient antiknock agent to bring its octane number to about 100.

CECIL L. BROWN.